

# United States Patent Office

2,935,401

Patented May 3, 1960

1

2,935,401

## CONTROL ROD ALLOY CONTAINING NOBLE METAL ADDITIONS

William K. Anderson and William E. Ray, Schenectady, N.Y., assignors to the United States of America as represented by the United States Atomic Energy Commission

No Drawing. Application December 10, 1957  
Serial No. 701,937

12 Claims. (Cl. 75—173)

This invention relates in general to alloys suitable for use in the fabrication of control rods for neutronic reactors, and more specifically to silver base alloys suitable for such applications.

It is an object of this invention to provide an alloy composition suitable for use in fabricating control rods for neutronic reactors.

It is a further object of this invention to provide an alloy composition suitable for use in control rods for neutronic reactors, which possesses superior structural strength properties.

The alloys of this invention are essentially improvements of an already existing alloy, which is the subject of copending application Ser. No. 688,995, filed October 8, 1957. This alloy is known to have nuclear properties which make it quite suitable for use as a neutronic reactor control rod material. The already known alloy consists essentially of from 0 to 10 percent of cadmium, from 2 to 20 weight percent of indium and from 65 to 85 weight percent silver, and while this alloy has a proven nuclear worth, it lacks structural strength characteristics to an extent sufficient to restrict its use in some applications.

It has been found that this shortcoming of the original cadmium-indium-silver alloy may be overcome through the addition to the basic alloy of a noble metal selected from the group consisting of platinum, ruthenium, rhodium, osmium, and palladium in amounts from about 0.5 weight percent to about 1.5 weight percent. This can be seen more clearly by reference to the attached table.

*Data showing mechanical properties of modified Cd—In—Ag alloys (additions of the indicated percentage of fourth metal, as shown, to the basic 5% Cd—15% In—80% Ag alloy)*

Any conventional method of preparation may be employed in producing the alloy compositions of this invention. The alloy can be easily prepared by placing in a graphite crucible the desired constituents. The 5 components may then be melted by means of induction heating apparatus or by any other suitable means. To prevent oxidation of the molten alloy, a protective cover of calcined coke pellets may be placed on the surface of the melt, and after melting, the alloy may be cast by any 10 convenient method.

It is not intended that this invention be limited in any way except by the scope of the appended claims.

We claim:

1. An alloy adapted for use as a neutronic reactor control rod material consisting of from 0.5 weight percent to about 1.5 weight percent of a noble metal selected from the group consisting of platinum, ruthenium, rhodium, osmium, and palladium, up to 10 weight percent of cadmium, from 2 weight percent to 20 weight percent indium, the balance being silver.
2. A control rod member for use in neutronic reactors consisting of an alloy falling within the compositions of claim 1.
3. An alloy adapted for use as a neutronic reactor control rod material consisting of about 1 weight percent platinum, about 5 weight percent cadmium, about 15 weight percent indium, the balance being silver.
4. A control rod member for use in neutronic reactors consisting of the alloy of claim 3.
5. An alloy adapted for use as a neutronic reactor control rod material consisting of about 1 weight percent ruthenium, about 5 weight percent cadmium, about 15 weight percent indium, the balance being silver.
6. A control rod member for use in neutronic reactors consisting of the alloy of claim 5.
7. An alloy adapted for use as a neutronic reactor control rod material consisting of about 1 weight percent rhodium, about 5 weight percent cadmium, and 15 weight percent indium, the balance being silver.
8. A control rod member for use in neutronic reactors consisting of the alloy of claim 7.
9. An alloy adapted for use as a neutronic reactor control rod material consisting of about 1 weight percent osmium, about 5 weight percent cadmium, about 15 weight percent indium, the balance being silver.

| Composition                                          | Sample Number | 0.2% Offset, Yield Str.,<br>lbs./in. <sup>2</sup> | Ult. Str.,<br>lbs./in. <sup>2</sup> | Percent Elong. | Percent Reduct.<br>of area | Hardness,<br>R <sub>x</sub> | Temp.   |
|------------------------------------------------------|---------------|---------------------------------------------------|-------------------------------------|----------------|----------------------------|-----------------------------|---------|
| Base Alloy—<br>(Cd 5 w/o, In 15 w/o, Ag<br>balance.) | 1             | 11,760                                            | 44,250                              | 78.2           | 57.3                       | 49.1                        | Rm.     |
|                                                      | 2             | 11,590                                            | 41,590                              | 71.8           | 59.5                       | 49.7                        | Rm.     |
|                                                      | 3             | 11,910                                            | 40,670                              | 75.0           | 61.4                       | 49.9                        | Rm.     |
|                                                      | 4             | 7,400                                             | 10,360                              |                | 60.5                       | 52.9                        | 600° F. |
| 0.05 wt. Percent Pt.                                 |               | 5,900                                             | 37,400                              | 84.4           | 59.7                       | 38                          | Rm.     |
| 0.1 wt. Percent Pt.                                  |               | 9,300                                             | 38,700                              | 81.2           | 61.6                       | 45                          | Rm.     |
| 0.5 wt. Percent Pt.                                  |               | 14,000                                            | 40,500                              | 75.0           | 57.8                       | 52                          | Rm.     |
| 1.0 wt. Percent Pt.                                  | 1             | 16,200                                            | 41,100                              | 65.6           | 51.0                       | 64                          | Rm.     |
| 1.0 wt. Percent Pt.                                  | 2             |                                                   | 15,200                              | 50.0           | 44.9                       | 64.1                        | 600° F. |
| 1.0 wt. Percent Pt.                                  | 3             | 11,800                                            | 14,750                              |                | 41.5                       | 63.5                        | 600° F. |
| 1.0 wt. Percent Pd.                                  | 1             | 20,490                                            | 43,800                              | 68.8           | 52.2                       | 60.9                        | Rm.     |
| 1.0 wt. Percent Pd.                                  | 2             | 20,390                                            | 43,790                              | 75.0           | 52.0                       | 55.9                        | Rm.     |
| 1.0 wt. Percent Ru.                                  | 1             | 18,990                                            | 38,690                              | 75.0           | 59.4                       | 37.9                        | Rm.     |
| 1.0 wt. Percent Ru.                                  | 2             | 10,930                                            | 12,830                              |                | 94.1                       | 37.5                        | 600° F. |
| 1.0 wt. Percent Ru.                                  | 3             | 18,660                                            | 33,160                              | 75.0           | 57.1                       | 36.9                        | Rm.     |
| 1.0 wt. Percent Ru.                                  | 4             | 11,170                                            | 12,680                              | 59.4           | 62.4                       | 48.9                        | 600° F. |
| 1.0 wt. Percent Ru.                                  | 5             | 21,010                                            | 39,760                              | 65.6           | 48.8                       | 50.9                        | Rm.     |
| 1.0 wt. Percent Ru.                                  | 6             | 11,500                                            | 13,240                              | 53.2           | 45.4                       | 54.4                        | 600° F. |
| 1.0 wt. Percent Os.                                  | 1             | 21,730                                            | 40,170                              | 56.2           | 46.3                       | 50.5                        | Rm.     |
| 1.0 wt. Percent Os.                                  | 2             | 21,910                                            | 39,360                              | 62.4           | 47.7                       | 64.2                        | Rm.     |
| 1.0 wt. Percent Rh.                                  | 1             | 26,610                                            | 44,070                              | 59.4           | 56.1                       | 73.9                        | Rm.     |
| 1.0 wt. Percent Rh.                                  | 2             | 26,700                                            | 44,170                              | 62.4           | 58.7                       | 70.7                        | Rm.     |
| 1.0 wt. Percent Rh.                                  | 3             | 26,550                                            | 44,600                              | 62.4           | 67.3                       | 74.8                        | Rm.     |
| 1.0 wt. Percent Rh.                                  | 4             | 11,560                                            | 13,760                              | 59.4           | 73.4                       | 74.9                        | 600° F. |
| 1.0 wt. Percent Rh.                                  | 5             | 11,150                                            | 12,840                              | 87.6           | 89.4                       | 75.4                        | 600° F. |
| 1.0 wt. Percent Rh.                                  | 6             | 10,880                                            | 12,260                              | 65.6           | 73.9                       | 77.0                        | 600° F. |

10. A control rod member for use in neutronic reactors consisting of the alloy of claim 9.

11. An alloy adapted for use as a neutronic reactor control rod material consisting of about 1 weight percent palladium, about 5 weight percent cadmium, about 15 weight percent indium, the balance being silver. 5

12. A control rod member for use in neutronic reactors consisting of the alloy of claim 11.

References Cited in the file of this patent

UNITED STATES PATENTS

2,157,933 Henzel et al. 1 May 9, 1939

OTHER REFERENCES

Technical Progress Review, Reactor Core Materials, vol. 1, No. 1, March 1958. (Pages 23 and 26 relied on.)